

1

3,184,304

## TUNGSTEN ALLOYS

George M. Andes, Wilmington, Del., assignor to E. I. du Pont de Nemours and Company, Wilmington, Del., a corporation of Delaware  
No Drawing. Filed Mar. 16, 1961, Ser. No. 96,075  
10 Claims. (Cl. 75—134)

This invention relates to high-temperature tungsten-base alloys containing chromium and titanium. These alloys may also contain as optional ingredients small amounts of iron, nickel, or cobalt.

Although tungsten possesses the highest melting point of all the metal elements, it suffers the disadvantage of being very susceptible to oxidation at elevated temperatures. For this reason, the use of tungsten as a high-temperature material has been somewhat limited. The present invention provides tungsten-base alloys having significantly improved oxidation resistance. It will be seen from data presented herein that as much as a 100-fold decrease in the rate of oxidation can be obtained with ternary tungsten-base alloys containing chromium and titanium within certain specified proportions. More specifically, it has been found that alloys containing about 20–40% by weight of chromium, about 1–25% by weight of titanium, about 0–10% by weight of a metal selected from the group consisting of iron, nickel, and cobalt, and combinations thereof, the balance being essentially tungsten in an amount of at least 45% by weight, are particularly resistant to oxidation at temperatures as high as 1200° C. As can be seen from the above ranges, the elements iron, nickel, and cobalt are optional elements which may or may not be present in the alloy composition. The table which appears hereinafter will show that excellent oxidation resistance can be obtained even when these elements are omitted from the alloy. Also, it should be pointed out that the 0–10% range for the iron group metals refers to the total weight of iron, nickel, and cobalt present.

In a preferred embodiment of this invention, the alloys comprise from 35%–40% by weight of chromium, about 1%–13% by weight of titanium, about 0%–10% by weight of metals from the group consisting of iron, nickel, and cobalt, the balance being essentially tungsten in an amount of at least 45% by weight.

Any of several well-known methods may be used to prepare the alloys of this invention. For example, they may be prepared by the arc melting of the metal constituents in powdered form. In preparing the alloys in this fashion, the metal powders are blended in the proper proportions and thoroughly mixed to yield the desired nominal composition. If desired, the mixture of metal powders may be compacted into small billets

2

before arc melting. Because of differences in melting points and in vapor pressures of the alloying elements at high temperatures, loss by volatilization or scattering of powders by the arc may thus be minimized. However, the powder mixture can be melted directly without compaction. In order to insure homogeneity of composition in the alloys, the mixture of metals should be melted several times, and preferably the casting turned over between melts.

For a clearer understanding of the invention, the following specific examples are given. These examples are intended to be merely illustrative of the invention and not in limitation thereof.

### EXAMPLE I

An alloy of tungsten, chromium, and titanium was prepared as follows:

A mixture of metal powders comprising 50 parts of tungsten, 40 parts of chromium, and 10 parts of titanium was thoroughly blended and compacted under a pressure of approximately 50 t.s.i. This compact was then arc melted under vacuum and cooled. The casting was turned over and remelted, the melting and cooling process being carried out four times to insure homogeneity in the sample.

The melted sample was analyzed and found to be 50% tungsten, 39% chromium, and 11% titanium by weight.

The specimen was weighed and placed in a furnace which was a part of a continuously recording thermobalance. A flow of dry air at a rate of 1000 cc./min. was directed over the sample and the specimen was held at a temperature of 1200° C. After five hours in the oxidizing atmosphere, the weight gain on the sample was found to be 5.3 mg./cm.<sup>2</sup>. The alloy sample was exposed to the oxidizing atmosphere at 1200° C. for a total of 42 hours. The initial rate of oxidation of the sample was found to be 2.8 mg./cm.<sup>2</sup>/hr., while the final rate after 42 hours was found to be 0.5 mg./cm.<sup>2</sup>/hr. The oxide film which formed on the sample was found to be very adherent.

A sample of pure tungsten was tested under the same conditions as the alloy sample. The initial rate of oxidation was found to be 150 mg./cm.<sup>2</sup>/hr. This rate did not diminish by the end of one hour of testing. The weight gain after five hours of oxidation testing was 296 mg./cm.<sup>2</sup>.

### EXAMPLES II THROUGH VII

Other alloys were prepared and tested in the same manner as the alloy of Example I. The composition of these alloys and the results of testing for resistance to oxidation and for rate of oxidation at 1200° C. are given in the following Table I.

Table I

|         | Alloy composition (analyzed), weight percent |      |      |     |     | Total hrs. at 1200° G. | Oxidation test results (Recording Thermobalance) in flowing air |                  |                                                                              |  |
|---------|----------------------------------------------|------|------|-----|-----|------------------------|-----------------------------------------------------------------|------------------|------------------------------------------------------------------------------|--|
|         | W                                            | Cr   | Ti   | Fe  | Ni  |                        | Oxidation rate                                                  |                  | Weight gain, mg./cm. <sup>2</sup> , after 5 hours unless otherwise specified |  |
|         |                                              |      |      |     |     |                        | Initial                                                         | Final            |                                                                              |  |
| Control | 100                                          |      |      |     |     | 5                      | 150                                                             | <sup>a</sup> 150 | 296                                                                          |  |
| Ex. 1   | Bal.                                         | 39   | 11   |     |     | 42                     | 2.8                                                             | <sup>b</sup> 0.5 | 5.3                                                                          |  |
| Ex. 2   | Bal.                                         | 27.2 | 12.8 |     |     | 50                     | 5.7                                                             | 0.6              | 11.3                                                                         |  |
| Ex. 3   | Bal.                                         | 38   | 10   |     |     | 68                     |                                                                 | <sup>b</sup> 0.2 | 10                                                                           |  |
| Ex. 4   | Bal.                                         | 27.6 | 24.5 |     |     | 66                     | 10                                                              | <sup>b</sup> 0.5 | 7.1                                                                          |  |
| Ex. 5   | Bal.                                         | 39.5 | 1.6  | 0.1 | 8.1 | 138                    | 2.2                                                             | <sup>b</sup> 0.2 | 4.5                                                                          |  |
|         | Bal.                                         | 39.5 | 1.6  | 0.1 | 8.1 | 96                     | 1.0                                                             | <sup>b</sup> 0.1 | 3.0                                                                          |  |
|         | Bal.                                         | 39.5 | 1.6  | 0.1 | 8.1 | 96                     | 1.8                                                             | 0.05             | 2.5                                                                          |  |
| Ex. 6   | Bal.                                         | 37.3 | 1.5  | 7.8 |     | 68                     |                                                                 | <sup>b</sup> 0.2 | 2.7                                                                          |  |
| Ex. 7   | Bal.                                         | 35.6 | 1.7  | 8.7 | 3.2 | 24                     |                                                                 |                  | <sup>c</sup> 253                                                             |  |

<sup>a</sup> After one hour. <sup>b</sup> The oxide scale on these samples was found to be especially adherent. <sup>c</sup> After 24 hours

Other methods may be used to prepare the alloys of this invention. One method which has frequently been employed to effect alloying of tungsten with other elements has been to prepare compacts of metal powders and to effect sintering of the compacted powder mix. A suggested method of compaction of metal powders is one in which the compaction is achieved by the carefully controlled detonation of an explosive charge. This explosive compaction of powder mixes has been very effectively employed in the preparation of dense compacts which are then sintered to effect alloying of the elements.

Another method which has been employed in the preparation of the tungsten-rich alloys of this invention is that of sealing uncompacted powder blends in stainless steel tubes. These tubes are heated to 1250° C. and then rolled and forged. This process yields alloy slabs of almost full density. The alloy systems of this invention are particularly well adapted to this rolling and forging technique. Since some of the alloying elements have considerable solubility for gases, porosity of the compact is minimized. The stainless steel tubes in which the metal powders are heated may be evacuated to minimize further the porosity of the compact.

The alloys of this invention were prepared using commercial metal powders of the highest purity available. Because of the extremely high melting point of tungsten and the high vapor pressures of chromium and titanium at the temperatures under which the alloys of this invention are prepared, it is sometimes difficult to prepare these alloys without loss of some amount of one or more of the alloying elements. The claims are therefore to be construed as defining the alloy compositions in parts by weight as determined by analysis.

The alloys of this invention are suitable as materials of construction in hot rolls for rolling mills. The alloys can also be used to manufacture furnace parts where strength at high temperature is needed and exposure to air or oxygen may be encountered. Also, the alloys may be fabricated into dies used in high-temperature extrusions and flame tips for gas burners.

Since it is obvious that many changes and modifications can be made in the above-described details without departing from the nature and spirit of the invention, it is to be understood that the invention is not to be limited to said details except as set forth in the appended claims.

The embodiments of the invention in which an exclusive property or privilege is claimed are defined as follows:

1. A high-temperature, oxidation-resistant alloy consisting essentially of about 20%–40% by weight of chromium, about 1%–25% by weight of titanium, and up to 10% by weight of a metal selected from the group consisting of iron, nickel, cobalt, and combinations thereof, the balance being essentially tungsten in an amount of at least 45% by weight.

2. A high-temperature, oxidation-resistant alloy consisting essentially of about 20%–40% by weight of chromium, about 1%–25% by weight of titanium, the balance being essentially tungsten in an amount of at least 45% by weight.

3. A high-temperature, oxidation-resistant alloy consisting essentially of about 35%–40% by weight of chromium, about 1%–13% by weight of titanium, and up to 10% by weight of a metal selected from the group consisting of iron, nickel, cobalt, and combinations thereof, the balance being essentially tungsten in an amount of at least 45% by weight.

4. A high-temperature, oxidation-resistant alloy consisting essentially of about 35%–40% by weight of chromium, about 1%–13% by weight of titanium, the balance being essentially tungsten in an amount of at least 45% by weight.

5. A high-temperature, oxidation-resistant alloy consisting essentially of, by weight, 39% chromium, 11% titanium, the balance being essentially tungsten.

6. A high-temperature, oxidation-resistant alloy consisting essentially of, by weight, 39.5% chromium, 1.6% titanium, 0.1% iron, 8.1% nickel, the balance being essentially tungsten.

7. A high-temperature, oxidation-resistant alloy consisting essentially of, by weight, 27.2% chromium, 12.8% titanium, the balance being essentially tungsten.

8. A high-temperature, oxidation-resistant alloy consisting essentially of, by weight, 37.3% chromium, 1.5% titanium, 7.8% iron, the balance being essentially tungsten.

9. A high-temperature, oxidation-resistant alloy consisting essentially of, by weight, 27.6% chromium, 24.5% titanium, the balance being essentially tungsten.

10. A high-temperature, oxidation-resistant alloy consisting essentially of, by weight, 38% chromium, 10% titanium, the balance being essentially tungsten.

#### References Cited by the Examiner

##### UNITED STATES PATENTS

|           |       |               |          |   |
|-----------|-------|---------------|----------|---|
| 1,471,326 | 10/29 | Copland       | 75—175.5 | X |
| 2,030,229 | 2/36  | Schwarzkopf   | 75—176   |   |
| 2,470,790 | 5/49  | Price         | 75—176   |   |
| 2,491,866 | 12/49 | Kurtz         | 75—176   |   |
| 2,850,385 | 9/58  | Nisbet        | 75—176   |   |
| 2,977,225 | 3/61  | Wlodek et al. | 75—176   |   |

##### FOREIGN PATENTS

|         |       |                |
|---------|-------|----------------|
| 550,648 | 12/57 | Canada.        |
| 741,360 | 3/52  | Great Britain. |

DAVID L. RECK, Primary Examiner.

RAY K. WINDHAM, Examiner.